

Aug. 2, 1927.

G. L. PREBLE

1,637,709

STIFFENER FOR BOOTS AND SHOES

Filed March 18, 1924

*Fig. 1*



*Fig. 2*



*Inv. no. 1,637,709*  
George L. Preble,  
by Tolbert, Tolbert & Cushman,  
attys.

Patented Aug. 2, 1927.

1,637,709

# UNITED STATES PATENT OFFICE.

GEORGE L. PREBLE, OF LYNN, MASSACHUSETTS, ASSIGNOR, BY DIRECT AND MESNE ASSIGNMENTS, TO PREBLE BOX TOE CO., OF LYNN, MASSACHUSETTS, A CORPORATION OF MASSACHUSETTS.

## STIFFENER FOR BOOTS AND SHOES.

Application filed March 18, 1924. Serial No. 700,009.

Heretofore it has been proposed to roll a thick gummy coating or spreading mixture upon a fibrous base for the purpose of making box-toes for boots and shoes. I have 5 discovered that markedly superior results can be secured by thoroughly impregnating a fibrous base with a liquid mixture contained in a volatile carrier, partially evaporating the carrier, compacting the mass of 10 fibers, and finally drying. Thus instead of producing a superficial coating by rolling I completely fill the interstices by impregnation and preferably scrape off the superficial excess.

15 Any fabric or felted base may be employed, depending upon the type of boot and shoe for which the stiffeners are intended, but I have secured best results with a fabric sheet (such as burlap for men's box-toes and 20 sheeting for women's box-toes) having anchored thereto a mass of loose fibers such as jute fibers. The fibers may be anchored in various ways but preferably by punching the fibers through the fabric at recurrent intervals.

In general the treatment of the base comprises impregnating with a fluid mixture containing a suitable compound or compounds of cellulose or its polymers partially 30 or completely dissolved in a suitable solvent, preferably with the addition of a comminuted fluid-retaining substance or an adhesive saccharose or both, saturating a fibrous base material with said mixture, shaping the 35 material so treated and permitting the same to harden, accompanied by evaporation of the solvent. The cellulosic compound used may be any appropriate derivative or compound of cellulose or a polymeric form of 40 cellulose, characterized by ability to form a crystalloidal or colloidal solution in a suitable solvent and to stiffen or harden a base material saturated therewith upon subsequent evaporation of the solvent. For some purposes, where the adhesive properties of the 45 molding composition are to be prolonged during the drying and hardening operations, it has been found advantageous to add to the impregnating fluid a saccharose or polysaccharose, such as sugar, dextrine, etc. The interaction or interrelation between such addition and the other ingredient or ingredients is not clear but it is observed that when this addition is made to the impregnating

55 fluid a larger amount of the solvent or of the comminuted material may be added thereto without decreasing the saturation properties of the mixture and its adhesive propensities with respect to other materials which it may be desirable to incorporate with 60 the molded article are enhanced.

The comminuted substance used may or may not be cementitious, but is of such character as to cling to the fibers of the base and to form capillary voids, adapted to induce absorption of the fluid therein and to retain a relatively large proportion of it within and upon the base material used. 65 The saturation of the base material is accomplished in any convenient manner as by 70 simply immersing it in the fluid, when rapid and complete impregnation of the material takes place. The superficial excess is preferably removed to provide the desired thickness and the treated material may be compressed and compacted into a thin dense sheet, or may be molded to the desired form 75 by any convenient means with or without pressure as the character of the stiffener or the purpose for which it is intended may 80 determine. The shaping operation may be effected after impregnation and before hardening, as described, or the material may be allowed to harden before being shaped and subsequently softened for the shaping operation, after which the material is allowed to 85 thoroughly dry and harden in its final form.

While the ingredients of the impregnating composition may be widely varied for different types of boots and shoes the following 90 proportions, which are well adapted to the principal uses, will serve as examples:

Women's box-toes: 16 vols. liquid celluloid (20° Bé.), 4 vols. comminuted asbestos, 1 vol. dry dextrine, 12 vols. alcohol.

Men's box-toes: 20 vols. liquid celluloid (20° Bé.), 4 vols. comminuted asbestos, 4 vols. comminuted plaster of Paris, 1 vol. dextrine, 16 vols. alcohol.

The celluloid, when incorporated in the base, renders the product stiff but elastic, and can readily be resoftened by wetting with alcohol for the purpose of reshaping the product. The comminuted absorptive substance facilitates the impregnation of the base, apparently by helping to hold the celluloid solution in the base until it dries since a solution of this composition evidences much 100 105

less tendency to flow out of the base after impregnation and before drying than does a celluloid solution containing no such substance. The admixture of absorptive substance also reduces the amount of celluloid required to give the desired degree of stiffness and body to the treated base.

Plaster of Paris also adds stiffness if employed in unhydrated form and if the impregnating solution contains some water in addition to the celluloid solvent. The plaster of Paris also reduces the flammability of the resulting product and if used in sufficient proportion it renders the product fire-proof. Asbestos also reduces the flammability of the product and owing to its fibrous character, even in comminuted form, it renders the product smoother and tougher.

The ratio between the asbestos and plaster of Paris may be adjusted to any point at or between the two extreme limits depending upon the particular use. Likewise the ratio between the cellulosic material and the absorptive substance may be widely varied to suit the requirements of different bases and different products. For example, by using all plaster of Paris as the absorptive substance and using as much plaster of Paris as liquid celluloid (by vol.) the stiffeners are substantially fire-proof.

Fig. 1 is a sectional view of the stiffener material in which 1 represents the threads of the fabric and 2 the fibers, the cellulosic matrix being represented by cross-hatching and the comminuted absorptive substance by stippling.

Fig. 2 illustrates one application of the invention in which 3 is a last, 4 an insole, 5 a welt, 6 the shoe lining, 7 the box-toe and 8 the upper. If the box-toe has been dried prior to the lasting operation it is rewet by dipping in alcohol or other suitable softener prior to its application to the last.

An outstanding feature of the product so obtained is the large amount of cellulosic material which is incorporated therewith both within the interstices of the fabric and upon the surfaces. Such concentration produces a stiff and strong article after it has been allowed to harden, even when thin fabrics are used or when a thick fabric is impregnated and compacted to narrow dimensions.

The saturated fabric produced in this manner possesses an appreciable degree of adhesiveness while wet, but upon drying this rapidly diminishes. By the addition of saccharose, such as sugar or dextrine, to the impregnating fluid, it is found that its adhesive properties are prolonged and that surfaces to which the sheets may be applied

or other materials incorporated with the mixture, are permanently retained thereby.

While the celluloid contained in an article made according to the process described is 65 intrinsically flammable, the finished article itself will be found to be appreciably less inflammable regardless of the combustible or non-combustible condition of the fibrous material used, and so far as ignition is concerned may be subjected to relatively high 70 temperatures with impunity. The structure formed by the comminuted substance protects the celluloid in this regard and also imparts strength and rigidity to the whole. 75

In some instances, where neither flammability nor the other properties incidental to the addition of the comminuted substance are required and where the adhesive properties of the saccharose is unnecessary, impregnation may be effected with the cellulosic solution alone. Other variations and modifications of the invention may, and ordinarily will be made in practice to adapt it to the numerous purposes for which it is clearly 80 appropriate, and to modify or control the relative degree of the several effects upon the finished product which may under given circumstances be required, but such variations are within the invention and to be regarded as contemplated by the following claims.

I claim:

1. Stiffeners for boots and shoes comprising interconnected fibers, an interlacing network of absorptive particles incorporated therewith, and a matrix consisting of a cellulose compound and a saccharose, contained within the interstices between said fibers and particles.

2. Stiffeners for boots and shoes comprising a fibrous sheet, an interlacing structure of a comminuted substance interspersed among the fibers thereof, and a matrix of a cellulose ester and a saccharose in the interstices between said fibers.

3. Stiffeners for boots and shoes comprising a fibrous sheet, powdered asbestos interspersed among the fibers thereof, and a matrix of cellulosic compound susceptible of 110 softening with an organic solvent in the interstices between said fibers and asbestos.

4. Stiffeners for boots and shoes comprising a fabric sheet, hydrated powdered asbestos interspersed among the fibers thereof, and a matrix of a cellulose ester in the interstices between said fibers and powdered asbestos.

Signed by me at Boston, Massachusetts, this 5th day of March, 1924.

GEORGE L. PREBLE.